

## UNITED STATES PATENT OFFICE

2,229,420

## UNHAIRING PROCESS

Wilhelm Neugebauer, Wiesbaden-Biebrich, Germany, assignor to Kalle & Co. Aktiengesellschaft, Wiesbaden-Biebrich, Germany

No Drawing. Application June 22, 1938, Serial No. 215,238. In Germany June 29, 1937

4 Claims. (Cl. 195—6)

The present invention relates to unhauling processes.

It is known to use sulphites for unhauling hides or skins. These bodies are used in combination with lime or other substance of alkaline reaction which has been applied either simultaneously with the sulphite or in a subsequent operation on the hide. It is also known to use the sulphites in combination with enzymes in the unhauling process.

The unhauling process of the present invention treats the hide or skin simultaneously or successively with a sulphite preferably an alkali metal sulphite and a suitable enzyme in aqueous solution. It has been found that the activity of the sulphite in this process can be enhanced by simultaneous use of a salt of a heavy metal. If, for example, softened felts are handled first with a sulphite solution containing an addition of a copper salt, and finally with a solution of a proteolytic enzyme the unhauling operation is easier than in the absence of the copper salt. The same unhauling effect can be produced in a shorter time or with a smaller proportion of enzyme in consequence of the presence of the copper salt. Somewhat small proportions of copper salt suffice for this purpose. Considerable effects are obtained, for example, when the treating liquor contains only 1 part of copper sulphate per 10,000 parts. Other heavy metal salts besides the copper salts affect the unhauling in the manner described, although the action of the various heavy metals is not equally powerful. Mercury salts come first in this matter. Silver salts may also be used. Also mixtures of several metal salts may be employed.

It is advantageous to use the heavy metal salt in the presence of a substance capable of forming a complex salt with the heavy metal salt or another substance which retains the metal salt in solution at a hydrogen-ion concentration whereat there would otherwise be precipitated an insoluble metal compound. Such substances are, for instance, albuminous bodies, amino acids, oxy acids, thiourea, pyrophosphates, nitrilotriacetic acid or the like. There may also be used directly complex salts of heavy metals.

As enzymes especially proteolytic enzymes obtained with the aid of bacteria or fungi may be used. Also pancreatic enzymes are suitable.

It is possible according to the invention to treat the hides or skins first with the solution of the sulphite containing the heavy metal salt and to treat them in a subsequent operation with the enzyme in the same bath or preferably after

rinsing in a separate bath. In many cases it may also be practical to add the enzyme at the beginning of the operation to the solution containing the sulphite and the heavy metal salt. This manner of operation is, however, less recommended. Since many enzymes are very sensitive to traces of heavy metals it may be preferable to use an addition which protects the enzyme against poisoning by metal, when enzymes and heavy metal salts are simultaneously present.

The enzyme solution is adjusted to a suitable pH value in known manner. Its temperature may vary within somewhat wide limits, for example, between about 5° and 30° C. In general the operation is best conducted at room temperature. The described pretreatment with a solution free from enzymes may be conducted at the same temperature.

The following examples illustrate the invention:

(1) Soaked calf skins or skins of other animals are handled for 20 hours at about 20° C. in a solution of 10 kg. of sodium sulphite, 10 kg. of sodium bicarbonate, .3 kg. of copper sulphate and 4 kg. of peptone per 1000 l. water. For prevention of putrefaction, .1 per cent of an active disinfectant, for example one prepared according to U. S. Patent 1,919,293 and known by the Trade-Mark "Preventol f.I." may be added to the solution. The skins are then rinsed for a short time and then left for about 20 hours in a bath at 20° C. and of the following composition: .7 kg. of a commercial enzyme preparation from *Bacillus mesentericus*, 10 kg. of sodium bicarbonate, 1 kg. of "Preventol f.I." and 1000 l. of water. The skins are then freed from hair. Instead of the peptone there may be used 10 kg. of aqueous ammonia solution of 15 per cent strength, or there may be substituted for the peptone a suitable amino acid, an amine, a salt of an oxy acid or thiourea; if desired this complex forming substance may be omitted. It is possible to treat about 100 kg. of skins with the described solutions.

(2) Soaked calf skins are treated for 20 hours at room temperature with a solution of 10 kg. of sodium sulphite, 10 kg. of sodium bicarbonate, .3 kg. of sodium nitrilotriacetate and .2 kg. of copper sulphate in 1000 l. of water to which has been added about .1 per cent of "Preventol f.I." After the sulphite bath the skins are rinsed for a short time and then immersed in an enzyme bath at 22° C. and of the following composition: .1 kg. of pancreatin, 10 kg. of sodium bicarbonate, 1 kg. of "Preventol f.I." and 1000 l. of water. The skins

remain in this bath for about 20 hours. Instead of the pancreatin another proteolytic enzyme may be used, for example an enzyme obtained with the aid of *Bacillus mesentericus*, *Aspergillus oryzae* or *Aspergillus flavus*.

(3) Soaked calf skins are handled for 20 hours at room temperature in 500 l. of water containing 5 kg. of sodium sulphite, 5 kg. of sodium bicarbonate, .05 kg. of mercuricacetate and 1 kg. 10 of sodium nitrilotriacetate. The skins are then rinsed and treated in a bath of the following composition: 500 l. of water, 5 kg. of sodium bicarbonate, .3 kg. of trypase from *Bacillus mesentericus* and .2 kg. of thymol. The skins 15 remain in this bath for about 15 hours.

(4) Soaked goat skins are handled for 20 hours at 20-25° C. in a solution of 10 kg. of sodium sulphite, 5 kg. of sodium bicarbonate, 3 kg. of sodium nitrilotriacetate and .3 kg. of copper sulphate in 1000 l. of water. The skins are then rinsed and transferred to an enzyme bath consisting of a solution of 1 kg. of a commercial proteinase preparation from *Bacillus mesentericus* and 5 kg. of sodium bicarbonate in 500 l. 20 25 of water.

(5) Soaked calf skins are treated for about 20-30 hours with a solution at 20-25° C. of 10 kg. of sodium sulphite, 10 kg. of sodium bicarbonate, 3 kg. of sodium nitrilotriacetate, .3 kg. 30 of copper sulphate and 1 kg. of a commercial proteinase preparation from *Bacillus mesentericus* in 1000 l. of water.

(6) The operation is conducted as described in Example 5, but instead of .3 kg. of copper sulphate .4 kg. of mercuric sulphate is used. Silver nitrate may also be used as the heavy metal compound.

(7) Soaked calf skins are treated for 48 hours at about 25° C. with a solution of 6 kg. of potassium sulphite, 3 kg. of sodium bicarbonate, .1 kg. 40 of mercuric chloride and .5 kg. of a disinfecting means in 500 l. of water. The skins are rinsed for half an hour and then handled for 24 hours at about 25° C. in a bath containing .5 kg. of 45 sodium bicarbonate, .25 kg. of a commercial enzyme preparation from *Bacillus mesentericus* and .5 kg. of a disinfecting means in 500 l. of water.

(8) Soaked calf skins are treated for 48 hours 50 at about 25° C. with a solution consisting of 3 kg. of sodium sulphite, 3 kg. of sodium bicarbonate, .15 kg. of silver nitrate, .5 kg. of a disinfecting means and 500 l. of water. After rinsing the skins are treated for 24 hours at about 25-30° C.

with a solution of 1 kg. of sodium bicarbonate, .5 kg. of a disinfecting means and .25 kg. of an enzyme preparation from *Bacillus subtilis* in 500 l. of water.

(9) Soaked calf skins or goat skins are handled for 24 hours at about 25° C. in a solution which consists of 3 kg. of sodium sulphite, 3 kg. of sodium bicarbonate, .1 kg. of mercuric chloride, 1 kg. of sodium butylnaphthalinsulphonate, .5 kg. of a disinfecting means and 500 l. of water. 10 The skins are then rinsed and then treated for 48 hours at about 25° C. with a bath which contains 1 kg. sodium bicarbonate, .1 kg. of pancreas preparation and .5 kg. of a disinfecting means in 500 l. of water. 15

(10) Soaked sheep skins are coated on the meat side with the equal weight of the following lime cream which contains 20% of wood flour as a thickening means: 100 l. of water, 1.2 kg. of sodium sulphite, 1.2 kg. of sodium bicarbonate, .08 kg. of mercuric chloride, 1.5 kg. of potash soap, .35 kg. of a disinfecting means and .35 kg. of an enzyme preparation from *Bacillus mesentericus*. The skins are laid with their meat sides one upon another and remain lying for 48 hours 25 at about 20-25° C.

I claim:

1. An unhairing process which comprises treating a hide or skin with an aqueous solution containing a water-soluble sulphite and a water-soluble salt of a metal selected from the group consisting of mercury, silver and copper and with an aqueous solution containing a proteolytic enzyme. 30

2. An unhairing process according to claim 1 35 wherein the said heavy metal salt is a complex salt.

3. An unhairing process which comprises treating a hide or skin with an aqueous solution containing an alkali metal sulphite and a water-soluble complex salt of a metal selected from the group consisting of mercury, silver and copper and with an aqueous solution containing a proteolytic enzyme. 40

4. An unhairing process which comprises treating a hide or skin with an aqueous solution containing a water-soluble sulphite and a water-soluble salt of a metal selected from the group consisting of mercury, silver and copper and treating the said hide or skin in a subsequent operation with an aqueous solution containing a proteolytic enzyme. 45 50

WILHELM NEUGEBAUER.